

# UNITED STATES PATENT OFFICE.

GEORGE W. DOWNS, OF NEWARK, NEW JERSEY, ASSIGNOR, BY MESNE ASSIGNMENTS, TO  
WILLIAM T. PLUM, OF NEWARK, NEW JERSEY.

## PAPER OR BOARD.

No. 818,740

Specification of Letters Patent. Patented April 20, 1909.

Application filed May 20, 1908. Serial No. 433,824.

To all whom it may concern:

Be it known that I, GEORGE W. DOWNS, a citizen of the United States, residing at Newark, in the county of Essex and State of New Jersey, have invented certain new and useful Improvements in Paper or Board, of which the following is a full, clear, and exact specification.

My invention relates to an improved paper or board, and has for its object to make an improved paper or board which can be produced quickly and economically, and which possesses many desirable qualities.

My improved paper or board is preferably made of spent hops, to wit, such hops as have been used by brewers and from the leaves of which the bitter properties have been extracted, by reason of the cheapness of such material, and I use the entire body of such hops, not only the leaves, but the seeds or kernels as well, and in the use of such seeds or kernels resides an important part of my invention, as I have found that such kernels contain a very large percentage of resinous matter, as well as an important percentage of cellulose, and that such kernels, when properly reduced, form an adhesive mixture of the nature of a paste which is useful as a binder in cementing together the fibers.

The paper or board produced by me from such spent hops is of a light porous character, quite thick for its weight, and of a springy, elastic character, thereby admirably fitting it for use where a board or paper having such qualifications is desired, for instance, as a carpet lining, for which use it may, if desired, be corrugated.

In producing my improved product, I take the spent hops preferably as they come from the breweries, usually in a moist or soaked condition, in which condition they are soft and easily reduced, and without any preliminary treatment by chemicals or machinery, deposit them in the usual Holland beating engine, where they are reduced in either hot or cold water, and from which they later pass through a Jordan or refining engine to the paper machine. This Jordan engine I

prefer to set so that the stock shall be reduced to a fine fiber, as thereby the seeds or kernels will also be correspondingly reduced and be most efficient as a cement. After reduction the pulp is passed on to the paper-making machine and there run into paper or board in the usual manner. Should it be deemed advisable, I may line either one or both sides of said product, in which latter case the said hop-board or paper would form merely the center, but its valuable properties would still be evident.

It is apparent that while for some purposes the spent hops will form a stock of sufficient strength to make a paper or board, if a stronger product be desired a proportion of stronger fiber, such as sulfite, jute, or suitable mixed papers may be added. The said spent hops, owing to the treatment which they have passed through at the breweries, are soft and quickly reduced to pulp, and I have found that they may be prepared in an hour or even less.

Old hops or damaged hops which are less valuable for brewers' use may also be used by me as well as spent hops, as they contain all necessary material for the manufacture of paper or board, and the kernel of such hops is equally well adapted to serve as a binder, but in the use of such old or damaged hops (which are not spent) a slightly longer time is required in the beating engine.

By the expression "seeds or kernels in substantially their natural condition," or "resinous matter in substantially its natural condition" in the claims, is meant that the seeds or kernels, and the resinous matter respectively, have not been neutralized with an alkaline solution.

What is claimed is:

1. A paper or board containing spent hops having the seeds or kernels minutely subdivided, but otherwise in substantially their natural condition and uniformly distributed throughout the body of the paper or board.

2. A paper or board containing spent hop leaves and a binder formed of hop seeds or kernels and the resinous matter of said

seeds or kernels in substantially its natural condition.

3. A paper or board containing the leaves of hop blossoms and a binder formed of hop seeds or kernels and the resinous matter of said seeds or kernels in substantially their natural condition.

In testimony whereof, I have hereunto set my hand in the presence of two subscribing witnesses.

GEORGE W. DOWNS.

Witnesses:

CHARLES A. SCHEUBER,  
BENJAMIN G. BAIN.